

# United States Patent Office

2,980,530

Patented Apr. 18, 1961

1

2,980,530

## METHOD OF PRODUCING NODULAR IRON

Lester C. Crome, West Alexandria, Ohio, assignor to The Dayton Malleable Iron Company, Dayton, Ohio, a corporation of Ohio

No Drawing. Filed Dec. 11, 1958, Ser. No. 779,544

16 Claims. (Cl. 75—130)

This invention relates to the production of gray iron castings having in the as-cast state graphitic carbon present therein in substantially nodular form, and more particularly to a process for producing such castings by the addition of a rare earth fluoride and a reducing agent therefor to the molten gray iron before pouring. This application is a continuation-in-part of my copending applications Serial No. 640,624, filed February 18, 1957, and Serial No. 641,870, filed February 25, 1957, now both abandoned.

Various methods are now known for producing from a gray iron mix a cast iron having, in the as-cast state and without subsequent treatment, all or a substantial part of the graphitic carbon present in the casting in so-called "nodular" form. Such iron is now conventionally known as "nodular iron" and as having a "nodular" microstructure with reference to the form in which the free or graphitic carbon is present in the finished casting. The term "nodular" is now conventionally understood to include truly spherulitic carbon nodules as well as other agglomerations of graphitic carbon which, while not being true spherulites, are still quite different from the flake form of graphitic carbon usually found in gray iron castings which are not "nodular." As is well-known, cast iron having a nodular microstructure possesses mechanical properties such as tensile strength, ductility, etc., substantially greater than a cast iron not having nodular microstructure even though produced from a molten mix having substantially equivalent composition.

Most, if not all, of the various methods known today for producing nodular iron comprise adding a minor proportion of a nodularizing agent to the molten mix shortly before pouring or casting the mix. Among the many such additive materials or, as herein referred to, nodularizing agents described in the literature and known to men skilled in this art, perhaps the most widely used are magnesium, misch metal, certain calcium compounds, and various mixtures, alloys, and combinations thereof.

As will be understood, many of these nodularizing agents include materials having a fairly high cost, and it is desirable that the amount of nodularizing agent added be kept as low as possible consistent with obtaining the desired mechanical properties in the finished casting in order to keep the cost of producing the castings as low as possible. Furthermore, the presence of sulphur in the molten iron mix in proportions conventionally obtained when the mix is originally melted in a cupola has been found to be somewhat inimical to the nodularizing action of some if not all nodularizing agents. Also, melting the iron mix in the well-known direct arc type of foundry apparatus may be found to produce a molten mix which is not particularly susceptible to nodularizing, perhaps as a result of the arc melting process on nitrogen in the atmosphere.

It is now well known that certain rare earth metals have the effect of controlling the precipitation of graphitic carbon in a gray iron mix into a so-called nodular or spherulitic form during cooling of the mix in a mold to produce a gray iron casting having the graphitic carbon therein in nodular or spherulitic form in the casting as cast and without further treatment. The characteristics of rare earth metals, however, are such that, as it is attempted to add the metals directly to a ladle of molten iron prior to pouring, only a portion of the added metal

2

is dissolved in the molten iron and remains effective during the cooling of the casting to produce the desired nodular microstructure. A substantial part of the added metal is lost, as far as its nodular inducing function is concerned, by oxidation or combining with other elements present in the mix.

Since the cost of the added nodular inducing agent may be a significant or substantial factor in the cost of producing nodular iron, it is desired to add the nodular inducing agent to the molten iron in such a way that a maximum amount of the added material will be effective for nodular microstructure formation.

According to this invention, it may be desired to have a preliminary treatment of the molten melt for increasing the susceptibility or responsiveness thereof to a nodularizing agent later to be added thereto, and such pretreatment is provided by treating the molten iron with a calcium slag reducing material prior to the addition of a nodularizing agent to the melt. As a further feature of this invention, a nodular inducing agent or nodularizing agent, such as one or more rare earth metals, is added to the molten iron in the form of a compound, preferably the fluoride, and a reducing agent for such fluoride, such as calcium silicide or calcium carbide, is also added to reduce the fluoride in situ in the molten mix for liberating the rare earth metal nodularizing agent for direct solution or incorporation into the molten iron with substantially less loss of the nodularizing agent by oxidation or combination with other elements as would be the case if the nodularizing agent were added to the molten mix originally in elemental or free metallic form.

One object of this invention is to provide a slag treatment for increasing the susceptibility of a molten iron mix to the nodularizing action of a nodularizing agent.

Another object of this invention is to provide a pretreatment slag composition for use in the production of nodular iron as a preliminary treatment to increase the susceptibility of a molten iron mix to nodularizing by a nodularizing agent.

A further object of this invention is to provide a process of the character described for producing iron castings having in the as-cast state a nodular microstructure by the addition to a molten gray iron mix of rare earth fluorides and a reducing agent therefor.

Another object of this invention is to provide a method of inducing rare earth metals into a molten iron mix for inducing therein a nodular microstructure on the molten iron.

A further object of this invention is to provide a combined additive or addition agent of a molten iron mix to produce upon reaction therein a nodular inducing agent effective to control precipitation of graphitic carbon in said mix into a nodular form.

Still another object of this invention is to provide a method for reducing rare earth fluorides in a molten iron mix for liberating in said mix rare earth nodular inducing metals for direct solution therein to control precipitation of graphitic carbon into a substantially nodular form.

Other objects and advantages of this invention will be apparent from the following description and the appended claims.

Satisfactory results have been obtained according to this invention by utilizing a slag made up of one or more calcium mineral materials and carbon with or without the addition of a fluxing material thereto. Among the calcium materials satisfactory for practicing this invention are included limestone, calcium silicide, calcium oxide, calcium carbide, calcium fluoride, and mixtures thereof, although practicing of this invention is not limited to these particular materials. As will be understood, however, there are a number of calcium materials which

produce the desired characteristics in the melt but, for other reasons, are not preferred. For example, calcium chloride apparently provides the desired metallurgical properties but, because of its deliquescent character, it is difficult to handle in that any moisture in the slag causes undesired if not dangerous effects during the addition thereof to the molten iron, and the sulphate and nitrate are not preferred because of the presence of sulphur and nitrogen therein.

The carbon can be added in a variety of forms such as coke, graphite, or calcium carbide, and a preferred fluxing material is calcium fluoride or fluorspar.

A preferred slag embodying and for practicing this invention comprises a combination of a calcium carbonate as limestone, calcium fluoride as fluorspar, and coke, and preferred proportions for these materials (by weight on the molten mix) are 3% limestone, 3/4% fluorspar and 1% coke.

The calcium slag materials of this invention are added to the molten iron mix after melting and a short time before the addition thereto of a nodularizing agent. If the nodularizing agent is added to the iron melt in a ladle—upon tapping the melt from the furnace and before casting the melt from the ladle into molds—satisfactory results are obtained by adding the calcium slag on top of the melt in the furnace and before tapping into the ladle. The slag is allowed to stay on the melt for a short time of the order of 10 to 20 minutes and the thus treated mix is tapped from the furnace into a ladle. It will be understood that the slag treatment according to this invention is appropriate for use with various gray iron mixes having various compositions susceptible of nodularizing as is now well understood in this art.

Whereas the mechanics of the effect produced by a calcium slag treatment embodying this invention are not known completely, it has been noted that such treatment has a pronounced influence on the susceptibility of the molten iron to the nodularizing action of a nodularizing agent. The effect appears to be more than merely desulphurizing, and it is believed to include a reducing effect resulting from the carbon present in the slag or oxygen in the molten mix which would otherwise react undesirably with the nodularizing agent. It is not believed, however, that this enhanced susceptibility is achieved by actual solution of the calcium slag in the molten mix to become an additional component thereof during pouring because the enhanced characteristics are obtained although very little if any of the calcium material is discernibly retained in the finished casting. That is, the enhanced results of this invention are obtained even when as little as less than .005% calcium is retained in the finished casting.

The calcium slag pretreatment of this invention should also be distinguished from the known use of certain calcium materials as nodularizing agents such as, for example, those referred to in Patent No. 2,662,820. This distinction becomes apparent when it is noted that the calcium slag treatment according to this invention, even when calcium silicide and calcium fluoride are included in the slag, does not occur under such conditions as would produce a nodular iron in the absence of an additional nodularizing agent. It also appears that the slag treatment has an influence on the properties of the molten mix by some mechanism other than the actual solution of the calcium or other materials in the mix. It has been noted, however, that the utilization of calcium fluoride as a fluxing material somewhat enhances the effect of calcium slags embodying this invention.

As perhaps suggestive of an explanation of the possible reactions involved, the following equations are noted:



It will be noted that the last two reactions indicated above are reversible, and this also suggests that the mechanism of the slag treatment according to this invention is of the solution of the calcium in the molten iron, perhaps only momentarily after which the calcium again comes out of solution, because, for example, of the above noted minute proportions of calcium retained in the casting.

As illustrative of the results achieved according to this invention, a number of substantially equivalent gray iron mixes were melted, giving a slag pretreatment and then nodularized and cast. These melts were made from a mixture of 80% of a pig iron containing approximately 0.88% silicon, 0.028% sulphur, 0.028% phosphorous, 0.26% manganese, and above 4% carbon; to which was added about 20% of "silvery" iron containing approximately 10% silicon. In each case the nodularizing agent was 0.8% of an alloy of 5% misch metal, 20% magnesium and 75% copper. For each run a sand casting was made in the form of a so-called "keel block" with two "coupons," one of which was immediately tested for ultimate tensile strength and elongation, while the other was maintained at about 1300° F. for about 8 hours before being tested.

The results of these illustrative runs indicate that satisfactory nodularization and enhanced physical properties were achieved with the molten mixes which had received the calcium slag pretreatment according to this invention by the addition of only 0.8% of the additive nodularizing alloy, whereas as much as 1.25% of the same alloy is necessary to give equivalent nodularizing results in such molten mixes which are not subjected first to the calcium slag pretreatment. Since the additive alloy is comparatively expensive and a substantial factor in the cost of production of nodular iron castings, this sharp reduction in the amount of alloy needed, achieved by the pretreatment according to this invention, is a substantial commercial factor in the production of nodular iron castings.

The following table sets forth the results in a number of these illustrative runs, showing the composition of the slag, the amount of time between the addition of slag and tapping of the mix into the ladle for the addition thereto of the nodularizing agent, as well as the results of the mechanical property tests on the casting immediately broken from the mold and that which were held at 1300° F. for about 8 hours before being tested:

| 50 | Slag                  | Time | AS Cast  |        | Held 8 hrs. |        |
|----|-----------------------|------|----------|--------|-------------|--------|
|    |                       |      | Ultimate | Elong. | Ultimate    | Elong. |
| 55 | none                  | 0    | 75,100   | 2.0    | 65,000      | 4.5    |
|    | Do                    | 20   | 68,800   | 0.5    | 58,600      | 2.5    |
|    | 2.0% limestone        | 10   | 91,200   | 5.5    | 73,300      | 22.0   |
|    | 2.0% coke             | 20   | 82,700   | 2.0    | 71,700      | 8.0    |
|    | 2.0% limestone        | 20   | 82,700   | 3.0    | 61,600      | 5.0    |
|    | 2.0% fluorspar        | 10   | 92,200   | 3.0    | 61,600      | 5.0    |
|    | 2.0% coke             | 20   | 94,800   | 1.5    | 69,900      | 22.0   |
| 60 | 2.0% fluorspar        | 10   | 87,300   | 6.0    | 76,100      | 14.5   |
|    | 2.0% coke             | 20   | 95,100   | 1.5    | 73,100      | 16.0   |
|    | 3.0% limestone        | 20   | 85,500   | 3.5    | 67,900      | 22.5   |
| 65 | 3.0% fluorspar        | 10   | 101,600  | 5.0    | 70,900      | 23.5   |
|    | 1.0% coke             | 20   | 108,400  | 3.5    | 74,200      | 19.5   |
|    | 3.0% limestone        | 20   | 95,100   | 3.0    | 68,200      | 8.5    |
| 70 | 3.0% fluorspar        | 10   | 80,100   | 12.5   | 70,400      | 20.0   |
|    | 2.0% CaC <sub>2</sub> | 20   | 96,000   | 3.5    | 74,100      | 14.5   |
|    | 1.0% limestone        | 20   | 95,100   | 3.0    | 68,200      | 8.5    |
|    | 1.0% coke             | 20   | 96,000   | 3.5    | 74,100      | 14.5   |

It will thus be apparent that a pretreatment and calcium slag compositions are provided according to this invention which substantially enhance the susceptibility of a molten gray iron mix to the effect therein of a nodularizing agent, and that the relatively inexpensive materials of the slags provide a substantial saving in the amount of costlier nodularizing agents which are used as well as being readily and conveniently added in the furnace prior to tapping the melt.

When the rare earth metals, such as cerium, misch metal, "didymium," and other such metals or mixtures of metals, are added to a molten gray iron mix to exercise their well-known function of controlling the precipitation of graphitic carbon therein into a nodular or spherulitic form, a substantial amount of the added metal is lost during or shortly after the addition as by oxidation, preferential combination with sulphur, and other causes, all of which remove or subvert some of the added metal and prevent or interfere with the nodular inducing function thereof. It has been discovered, however, that, according to this invention, the rare earth metals may be added to a molten iron mix in the form of a compound which will prevent or minimize loss of the metal during addition. After addition to the mix, then, this compound can be reduced by the action of an added reducing agent to yield the rare earth metal itself for direct solution into the molten iron.

As will be understood, of course, a number of possible reactions may occur when a rare earth metal and/or a compound thereof is added to a molten iron mix at elevated temperatures, and, when rare earth compounds are added to molten iron mixes, the resulting reactions will depend in large measure on such thermodynamic consideration as heats of formation and free energies of the various reacting compounds. As based on such considerations, rare earth compounds and reducing agents can be selected so that, upon adding to molten iron in the presence of a reducing agent, the heats of formation and free energies of compounds which might result from the interaction of the added materials will favor the reduction of the rare earth metal compound to the free metal in the mix. In such an environment the reaction involved will preferentially approach as an end point the production of that one of the several possible resultant compounds which has the highest heat of formation and the lowest free energy. Since the rare earth fluorides have lower heats of formation than calcium fluoride, the desired reduction takes place.

Accordingly, in a situation where calcium has an opportunity to reduce cerium fluoride, the energy conditions such as the relative heats of formation will encourage the replacement of cerium by calcium, thereby reducing cerium fluoride to the metallic state as desired.

With the foregoing considerations in mind, it will be noted that the fluorides of the various rare earth metals and mixtures thereof all have heats of formation of an order of magnitude with respect to calcium fluoride so that any of the rare earth fluorides and mixtures thereof will be reduced by or replaced by calcium to liberate the metal when reacted in a molten iron mix.

According to this invention, then, rare earth metals in the form of the fluorides are added to a molten iron mix for reduction therein by a reducing agent containing calcium. Calcium silicide is preferred as a reducing agent and better results are obtained with calcium silicide than with other calcium materials. Also calcium itself has nodularizing properties, and some of the calcium may have its own effect in the iron during the course of the reducing reaction. Commercial grade calcium silicide usually contains approximately 30% calcium and 60% silicon, and this commercial grade of calcium silicide has been found satisfactory. It is such a material that is to be understood in the following examples when calcium silicide is mentioned.

Although many metallic elements are now known

to have a nodular inducing effect when added to molten iron, the rare earth elements for the process of this invention have been found most satisfactory. They may be used individually as fluoride or, as preferred from

5 a practical standpoint, as mixtures of fluorides. Of the various rare earth materials, misch metal is most readily available. As is well known, misch metal contains approximately 45% to 50% cerium with substantial proportions of lanthanum, praseodymium, neodymium, 10 and minor proportions of other rare earths. Both misch metal in metallic form and a mixture of rare earth fluorides (hereinafter sometimes referred to as misch metal fluorides) are available commercially. The fluorides may be produced from monazite ore which contains some or all of about 14 rare earth metals. In 15 processing the ore, which is principally a source of thorium, the various rare earth elements are readily converted to sulfates and thence to fluorides in known manner.

20 In addition to some possible assistance in nodular formation achieved by using calcium in the reducing agent, the calcium is also preferred by virtue of its position with respect to cerium in the chemical activity series and as a further driving force, along with other considerations as the heats of formation, to urge the desired reducing reaction preferentially to completion or other possible reactions which might occur with the same reactants. Thus, calcium is above cerium in the activity

25 series and separated therefrom by beryllium, thorium, magnesium, barium, strontium, and aluminum. In considering these other materials above cerium as possible components of the reducing agent, it is noted that beryllium is not satisfactory because of the almost inevitable formation of the very toxic beryllium oxide at the temperatures encountered with a molten iron mix. As a practical matter thorium is not preferred because of its presently limited availability for uses other than those connected with atomic energy developments as well as because of its greater usefulness for other purposes.

30 Magnesium is a well-known nodular inducing agent in its own right, and it would appear practically and commercially pointless to attempt to use it here as a reducing agent. Although barium and strontium are operative with this invention, the cost and lack of commercial 35 availability of appropriate compounds thereof indicate that these elements are not preferred, and aluminum, perhaps because of its being so close to cerium in the activity series, does not give practically satisfactory results.

40 50 Satisfactory results have been achieved according to this invention using various combinations of proportions of calcium silicide and misch metal fluoride. From the standpoint of efficiency and practical yield of nodular inducing agent, the proportions of from 2 to 4 parts of

55 calcium silicide to 1 part of rare earth fluoride are preferred, and satisfactory results have been achieved by adding from 0.5% to 3%, and preferably 1% to 2%, of such a mixture of calcium silicide and rare earth fluorides to the ladle of molten iron.

60 65 As illustrative of a process embodying this invention, the following examples are noted:

#### Example I

A charge of pig iron analyzing approximately

|            | Percent |
|------------|---------|
| Carbon     | 4.46    |
| Silicon    | 1.96    |
| Sulphur    | 0.021   |
| Phosphorus | 0.023   |
| Manganese  | 0.13    |

70 75 was melted with an additional 0.50% silicon. To the molten mix in the ladle before pouring was added 1.25% of a mixture of 4 parts calcium silicide to 1 part misch metal fluoride. Casting in the form of the well-known "keel

block" were cast in a sand mold. One was shaken out of the mold when solidified and tested for its various physical properties. This casting showed a Brinell number of 235, tensile strength of 95,700 pounds and an elongation of 6%. Each of these values being determined according to the standard metallurgical procedures for iron castings. Another casting poured from the same ladle was allowed to cool in the mold overnight and, when tested, showed a Brinell number of 170, tensile strength of 73,200 pounds and an elongation of 22%.

As illustrative of other reducing agents, runs were made achieving satisfactory results with calcium carbide as the reducing agent. One such run is noted here:

*Example II*

A pig iron charge analyzing

|            | Percent |
|------------|---------|
| Carbon     | 4.46    |
| Silicon    | 1.96    |
| Sulphur    | 0.021   |
| Phosphorus | 0.023   |
| Manganese  | 0.17    |

was melted with an additional 1% silicon. To the melted charge in the ladle was added 4% of a mixture of 2 parts calcium carbide and 1 part misch metal fluoride, and the melt was cast in a sand mold. The resultant casting, upon testing, had a Brinell number of 179, tensile strength of 70,300 pounds and an elongation of 8%.

A further commercial scale run embodying this invention is also noted:

*Example III*

A 9,000 pound charge of pig iron analyzing

|            | Percent |
|------------|---------|
| Carbon     | 4.34    |
| Silicon    | 1.91    |
| Sulphur    | 0.024   |
| Phosphorus | 0.026   |
| Manganese  | 0.17    |

was melted and heated to approximately 2800° F. at which time 1.2% additional silicon was added from 75% ferrosilicon. A slag of 2% lime, 0.75% fluorspar, and 1% petroleum coke was then added to the furnace and held for 20 minutes, after which 2000 pounds of the mix was tapped into a ladle and 1% of a mixture of 4 parts calcium silicide to 1 part misch metal fluoride was added. A 1" keel block cast from this ladle tested to have a Brinell number of 174, ultimate tensile strength of 71,700 pounds and an elongation of 20%.

It should be noted, as will be understood by men skilled in the art, that for castings in which a predominately pearlitic structure is desired, tensile strengths of in excess of 80,000 pounds and elongations of in excess of 2% are achieved according to this invention, while, with castings in which a predominately ferritic structure is produced, tensile strengths of in excess of 60,000 pounds with elongations of 10% or more are achieved.

It should also be noted that the various methods heretofore devised for extending the effective time of rare earth type nodular inducing agents in a molten mix and methods heretofore devised for otherwise enhancing the yield or effectiveness of such agents are applicable to methods embodying this invention, since the function of inducing graphite precipitation into a nodular form is achieved with this invention by the rare earth metals liberated in the molten mix from the reduction of the added compound, and the mechanism of such graphite precipitation is believed to be substantially the same as if the elemental metal were added as such to the molten mix instead of being produced therein by reduction of a compound of the metal.

As mentioned above, however, the use of a calcium compound as the reducing agent probably contributes its

own part in the nodular microstructure formation as disclosed, for example, in Patent No. 2,662,820. Generally substantially the same considerations as to the length of time before pouring during which the nodular reducing agent will remain effective in the molten metal are obtained with processes obtaining this invention as with other nodular iron processes in which rare earth metals are added as such to the molten mix.

Also, in view of the nodularizing effect of calcium or calcium silicide, it will be apparent that, as the proportion of fluoride in the added mixture is decreased, the proportion of calcium silicide must be increased to obtain the desired completeness of nodularization from the additive. Since in many instances it may not be desired so to increase the calcium silicide addition because, for example, of the other effects which additions of this material produce in molten iron. The preferred ranges are as set forth above—i.e., 2 to 4 parts of calcium silicide for each part of rare earth fluoride. These proportions may be varied, however, within wide ranges and considering that, for the reduction reaction to be efficient, a sufficient excess of the reducing agent must be present, and alternatively, sufficient fluoride should be used to achieve nodularizing without having to add an undesirably high amount of calcium silicide. That is, there appears to be a definitely cooperative and synergistic interaction between the fluoride and calcium additives. The reactions may be considered as first having the fluoride flux the calcium material in the solution where some of it then reduces the fluoride to provide rare earth metals for nodularizing while other of the calcium material may have its own nodularizing effect after being fluxed in the solution by the fluoride.

Although, as will be understood, it is quite possible to obtain nodular microstructures in castings in accordance with this invention and utilizing various types of iron mixes without such a preliminary calcium slag pretreatment, in commercial operations more satisfactory results are achieved by the pretreatment of the iron mix, in accordance with said copending applications prior to the addition of the nodularizing agent materials in accordance with this invention, and such more satisfactory results are most emphatically demonstrated in connection with the fact that the pretreatment steps appear to provide additional assurance that the desired nodular microstructure and enhanced physical properties will be routinely obtained time after time with all the castings poured from a particular melt or a particular ladle and without the commercially or economically undesirable question or possibility that, in some cases, a few castings from one heat or one pouring may, for reasons of variations in the melt during pouring, etc., fail to achieve the desired nodular microstructure.

While the methods, compositions and products described herein constitute preferred embodiments of the invention, it is to be understood that the invention is not limited to these precise methods, compositions and products, and that changes may be made therein without departing from the scope of the invention which is defined in the appended claims.

What is claimed is:

1. In the production of as-cast nodular iron from a molten gray iron mix by the use of rare earth metals as the nodularizing agent added to said molten mix, the method of increasing the efficiency of incorporation of said agent into said mix and of decreasing the amount of said agent added to said mix and the amount of said agent lost during said addition which comprises the steps of preparing a molten gray iron mix, treating said mix with a slag material comprising calcium carbonate and a carbonaceous material and calcium fluoride for enhancing the responsiveness of said mix to the effect of said nodularizing agent, thereafter adding to said mix before casting a rare earth metal fluoride and a reducing agent therefor, effecting reduction of said rare earth metal flu-

ride to said rare earth metal by said reducing agent in said molten mix for nodularizing action therein, and pouring the thus treated mix into a mold to form said casting.

2. In the production of as-cast nodular iron from a molten gray iron mix by the use of rare earth metals as the nodularizing agent added to said molten mix, the method of increasing the efficiency of incorporation of said agent into said mix and of decreasing the amount of said agent added to said mix and the amount of said agent lost during said addition which comprises the steps of preparing a molten gray iron mix, treating said mix with a slag material comprising calcium carbonate and a carbonaceous material for enhancing the responsiveness of said mix to the effect of said nodularizing agent, thereafter adding to said mix before casting a rare earth metal fluoride and a calcium reducing agent therefor, effecting reduction of said rare earth metal fluoride to said rare earth metal by said reducing agent in said molten mix for nodularizing action therein, and pouring the thus treated mix into a mold to form said casting.

3. In the production of as-cast nodular iron from a molten gray iron mix by the use of rare earth metals as the nodularizing agent added to said molten mix, the method of increasing the efficiency of incorporation of said agent into said mix and of decreasing the amount of said agent added to said mix and the amount of said agent lost during said addition which comprises the steps of preparing a molten gray iron mix, treating said mix with a slag material comprising calcium carbonate and a carbonaceous material for enhancing the responsiveness of said mix to the effect of said nodularizing agent, thereafter adding to said mix before casting a rare earth metal fluoride and calcium silicide as a reducing agent therefor, effecting reduction of said rare earth metal fluoride to said rare earth metal by said reducing agent in said molten mix for nodularizing action therein, and pouring the thus treated mix into a mold to form said casting.

4. In the production of as-cast nodular iron from a molten gray iron mix by the use of rare earth metals as the nodularizing agent added to said molten mix, the method of increasing the efficiency of incorporation of said agent into said mix and of decreasing the amount of said agent added to said mix and the amount of said agent lost during said addition which comprises the steps of preparing a molten gray iron mix, treating said mix with a slag material comprising calcium carbonate and a carbonaceous material for enhancing the responsiveness of said mix to the effect of said nodularizing agent, thereafter adding to said mix before casting a rare earth metal fluoride and calcium silicide as a reducing agent therefor, in the proportions of 2-4 parts of silicide to 1 part of fluoride, effecting reduction of said rare earth metal fluoride to said rare earth metal by said reducing agent in said molten mix for nodularizing action therein, and pouring the thus treated mix into a mold to form said casting.

5. In the production of as-cast nodular iron from a molten gray iron mix by the use of rare earth metals as the nodularizing agent added to said molten mix, the method of increasing the efficiency of incorporation of said agent into said mix and of decreasing the amount of said agent added to said mix and the amount of said agent lost during said addition which comprises the steps of preparing a molten gray iron mix, treating said mix with a slag material comprising calcium carbonate and coke for enhancing the responsiveness of said mix to the effect of said nodularizing agent, thereafter adding to said mix before casting  $\frac{1}{2}\%$  to 3% of a mixture of a rare earth metal fluoride and calcium silicide as a reducing agent therefor, effecting reduction of said rare earth metal fluoride to said rare earth metal by said reducing agent in said molten mix for nodularizing action therein, and pouring the thus treated mix into a mold to form said casting.

6. In the production of as-cast nodular iron from a molten gray iron mix by the use of rare earth metals as the nodularizing agent added to said molten mix, the method of increasing the efficiency of incorporation of said agent into said mix and of decreasing the amount of said agent added to said mix and the amount of said agent lost during said addition which comprises the steps of preparing a molten gray iron mix, treating said mix with a slag material comprising calcium carbonate and coke for enhancing the responsiveness of said mix to the effect of said nodularizing agent, thereafter adding to said mix before casting 1% to 2% of a mixture of a rare earth metal fluoride and calcium silicide as a reducing agent therefor, effecting reduction of said rare earth metal fluoride to said rare earth metal by said reducing agent in said molten mix for nodularizing action therein, and pouring the thus treated mix into a mold to form said casting.

7. In the production of as-cast nodular iron from a molten gray iron mix by the use of rare earth metals as the nodularizing agent added to said molten mix, the method of increasing the efficiency of incorporation of said agent into said mix and of decreasing the amount of said agent added to said mix and the amount of said agent lost during said addition which comprises the steps of preparing a molten gray iron mix, treating said mix with a slag material comprising calcium carbonate and coke for enhancing the responsiveness of said mix to the effect of said nodularizing agent, thereafter adding to said mix before casting  $\frac{1}{2}\%$  to 3% of a mixture of a rare earth metal fluoride and calcium silicide as a reducing agent therefor in the proportions of 2-4 parts silicide to 1 part fluoride, effecting reduction of said rare earth metal fluoride to said rare earth metal by said reducing agent in said molten mix for nodularizing action therein, and pouring the thus treated mix into a mold to form said casting.

8. In the production of as-cast nodular iron from a molten gray iron mix by the use of rare earth metals as the nodularizing agent added to said molten mix, the method of increasing the efficiency of incorporation of said agent into said mix and of decreasing the amount of said agent added to said mix and the amount of said agent lost during said addition which comprises the steps of preparing a molten gray iron mix, treating said mix with a slag material comprising calcium carbonate, coke and fluorspar for enhancing the responsiveness of said mix to the effect of said nodularizing agent, thereafter adding to said mix before casting 1% to 2% of a mixture of a rare earth metal fluoride and calcium silicide as a reducing agent therefor in the proportions of 2-4 parts silicified to 1 part fluoride, effecting reduction of said rare earth metal fluoride to said rare earth metal by said reducing agent in said molten mix for nodularizing action therein, and pouring the thus treated mix into a mold to form said casting.

9. In a method of the character described for producing nodular cast iron by a ladle addition of a nodularizing agent to a molten iron mix, the pre-treatment steps which comprise adding a slag including calcium carbonate and carbonaceous reducing material to said molten mix prior to ladle addition of said nodularizing agent, tapping said thus treated mix into a ladle after a predetermined short length of time effective for diffusion of said calcium slag through said mix, and then making said ladle addition of said nodularizing agent.

10. In a method of the character described for producing nodular cast iron by a ladle addition of a nodularizing agent to a molten iron mix, the pre-treatment steps which comprise adding a reducing slag including limestone and coke to said molten mix prior to ladle addition of said nodularizing agent for removal of sulphur and oxygen from said mix and otherwise enhancing the susceptibility thereof to said nodularizing agent, tapping said thus treated mix into a ladle after a predetermined

short length of time effective for diffusion of said slag through said mix, and then making said ladle addition of said nodularizing agent.

11. In a method of the character described for producing cast iron having in the as-cast state graphitic carbon present in nodular form, the steps which comprise forming a molten iron mix, adding to said mix before pouring a slag of limestone, carbon, and fluorspar, thereafter adding to said mix a nodularizing agent, and casting said thus treated mix.

12. In a method of the character described for producing nodular cast iron by a ladle addition of a nodularizing agent to a molten iron mix, the pretreatment steps for increasing the responsiveness of said molten iron mix to said nodularizing agent which comprises adding to said molten iron mix prior to said ladle addition of said nodularizing agent a slag comprising a mixture of carbonaceous material and a calcium carbonate material, holding said thus treated mix with said slag added thereto for a predetermined short length of time effective for diffusion of said slag through said mix, and then making said ladle addition of said nodularizing agent to said thus treated mix prior to casting said mix.

13. In a method of the character described for producing nodular cast iron by a ladle addition of a nodularizing agent to a molten iron mix, the pretreatment steps for increasing the responsiveness of said molten iron mix to said nodularizing agent which comprise adding to said molten iron mix prior to said ladle addition of said nodularizing agent a slag comprising a mixture of limestone and coke, holding said thus treated mix with said slag added thereto for a predetermined short length of time effective for diffusion of said slag through said mix, and then making said ladle addition of said nodularizing agent to said thus treated mix prior to casting said mix.

14. In a method of the character described for producing nodular cast iron by a ladle addition of a nodularizing agent to a molten iron mix, the pretreatment steps for increasing the responsiveness of said molten iron mix to said nodularizing agent which comprise adding to said molten iron mix prior to said ladle addition of said nodularizing agent a slag comprising a mixture of limestone, fluorspar and coke, holding said thus treated mix with said slag added thereto for a predetermined short length of time effective for diffusion of said slag through said mix, and then making said ladle addition of said nodularizing agent to said thus treated mix prior to casting said mix.

10

15

20

25

30

35

40

45

mined short length of time effective for diffusion of said slag through said mix, and then making said ladle addition of said nodularizing agent to said thus treated mix prior to casting said mix.

15. In a method of the character described for producing nodular cast iron by a ladle addition of a nodularizing agent to a molten iron mix, the pretreatment steps for increasing the responsiveness of said molten iron mix to said nodularizing agent which comprise adding to said molten iron mix prior to said ladle addition of said nodularizing agent a slag comprising a mixture of 3% limestone, 3/4% fluorspar and 1% coke by weight on said mix, holding said thus treated mix with said slag added thereto for a predetermined short length of time effective for diffusion of said slag through said mix, and then making said ladle addition of said nodularizing agent to said thus treated mix prior to casting said mix.

16. In a method of the character described for producing nodular cast iron by a ladle addition of a nodularizing agent to a molten iron mix, the pretreatment steps for increasing the responsiveness of said molten iron mix to said nodularizing agent which comprise adding to said molten iron mix prior to said ladle addition of said nodularizing agent a slag comprising a mixture of carbonaceous reducing material and a calcium mineral compound selected from the group consisting of the carbonate, silicide, halide, oxide, and mixtures thereof, holding said thus treated mix with said slag added thereto for a predetermined short length of time effective for diffusion of said slag through said mix, and then making said ladle addition of said nodularizing agent to said thus treated mix prior to casting said mix.

#### References Cited in the file of this patent

#### UNITED STATES PATENTS

|           |                    |               |
|-----------|--------------------|---------------|
| 170,420   | Warner             | Nov. 23, 1875 |
| 2,750,284 | Ihrig              | June 12, 1956 |
| 2,779,675 | Vennerholm         | Jan. 29, 1957 |
| 2,794,731 | Keizo Iwase et al. | June 4, 1957  |
| 2,821,473 | Moore              | Jan. 28, 1958 |
| 2,865,735 | Timmerbeil et al.  | Dec. 23, 1958 |

#### FOREIGN PATENTS

|         |               |               |
|---------|---------------|---------------|
| 203,754 | Australia     | Oct. 16, 1956 |
| 670,245 | Great Britain | Apr. 16, 1952 |

UNITED STATES PATENT OFFICE  
CERTIFICATE OF CORRECTION

Patent No. 2,980,530

April 18, 1961

Lester C. Crome

It is hereby certified that error appears in the above numbered patent requiring correction and that the said Letters Patent should read as corrected below.

Column 6, line 75, for "Casting" read -- Castings --; column 7, line 22, in the table of Example 2, right-hand column, for "0.17" read -- 0.13 --; column 11, line 15, for "comprises" read -- comprise --.

Signed and sealed this 19th day of September 1961.

(SEAL)

Attest:

ERNEST W. SWIDER

Attesting Officer

DAVID L. LADD  
Commissioner of Patents  
USCOMM-DC